

J. M. J. DEBOURG.

PROCESS FOR CONVERTING VEGETABLE FIBERS INTO THREADS OF SILKY APPEARANCE.  
APPLICATION FILED MAY 16, 1911.

1,018,650.

Patented Feb. 27, 1912.



WITNESSES:

John C. Sanders  
Arthur S. Peart

INVENTOR:

By Jean Marie Joseph Debourg.  
J. M. Debourg  
Wm. Wallace Black  
ATTY.

# UNITED STATES PATENT OFFICE.

JEAN MARIE JOSEPH DEBOURG, OF LYON, FRANCE.

## PROCESS FOR CONVERTING VEGETABLE FIBERS INTO THREADS OF SILKY APPEARANCE.

1,018,650.

Specification of Letters Patent. Patented Feb. 27, 1912.

Application filed May 16, 1911. Serial No. 627,561.

*To all whom it may concern:*

Be it known that I, JEAN MARIE JOSEPH DEBOURG, a citizen of the French Republic, residing at Lyon, in France, have invented 5 a certain new and useful Improvement in Processes for Converting Vegetable Fibers into Threads of Silky Appearance, of which the following is a specification.

The object of the invention is a process 10 for converting into silky threads, vegetable fibers such as flax, hemp, ramie and nettle.

The vegetable materials in the form of twists, plaits, branches or other form according to their nature, are first placed in 15 a boiling apparatus being then heated in two successive alkaline baths and washed. The materials are then carded, combed and spun, according to the use for which they are destined.

20 The annexed drawing shows as an example a boiler suitable for heating the materials, the figure being a vertical section of such boiler.

a designates a cylindrical boiler closed by 25 a hinged steam-tight lid b, and secured by pivoted pins c. A cage d having a transparent cover is arranged in the interior of the boiler and contains a number of superposed receptacles e e containing the materials to be treated. The said receptacles, 30 only two of which are represented in the drawing, are shaped like shallow circular trays and made of perforated metal. They rest one on the other and are provided at the center with an opening for passage of the vertical arm of a coil f. The said coil which ends in a cock g outside the apparatus makes several turns in the interior of the boiler, around the cage d and then passes 35 vertically upward at the axis of the apparatus. The coil is provided throughout its length with a quantity of small holes, which allow steam admitted through the cock g to escape into the liquid for the baths, and to 40 heat them to the desired temperature. The apparatus is completed by a drain cock h, a pressure gage i, a water-gage j, and, if necessary, one or more safety-valves k.

The method of operation is as follows:— 45 The trays e are charged separately with the materials to be treated, care being taken not to completely fill same, in order to allow for expansion and to permit them to be easily penetrated by the bath. The trays are then

placed one above the other in the interior of 55 the cage d and the whole is placed in the boiler a. A bath is then introduced into the boiler, composed of a solution of carbonate of soda of about 5-6 kgs. to 1000 liters of water. The boiler is then closed and the 60 bath heated for about two hours to a temperature of 120° centigrade to 130° centigrade corresponding to 2 or 3 atmospheres. This bath is drained off and replaced by another bath containing, to 100 liters of 65 water;

|                    |     |              |
|--------------------|-----|--------------|
| Slaked lime        | 108 | kilogr.      |
| Bisulfite of soda  | 5   | " 250 grams. |
| Sal-ammoniac       | 5   | " 500 "      |
| Peroxid of sodium  | 0   | " 560 " 70   |
| Salts of magnesium | 5   | " 750 "      |

After having closed the boiler, the bath is heated for about two hours, and then emptied away and replaced by ordinary tepid 75 water heated to 30° centigrade, to effect a primary rinsing. The material treated as above described is then removed from the boiler and placed in a bath of water acidulated by 1% of hydrochloric acid; in which 80 it is agitated quickly for 15 to 20 minutes, the material being then finally rinsed with ordinary fresh water. Materials thus treated can then be subjected to all the operations of carding, combing, spinning, dyeing, 85 etc., necessitated by their nature or purpose. Those materials which are to be of light colors can be bleached. The cleanliness and brilliancy of the threads which may have been tarnished by these processes can be 90 restored by treating them again slightly in a similar manner.

It should be understood that the proportions indicated above can vary within certain limits according to the material under 95 treatment, and the chemicals can be replaced by others in certain cases where the chemical composition will act better on the materials.

What I claim as my invention and desire to secure by Letters Patent of the United 100 States is:—

1. A process for converting vegetable fibers into threads of silky appearance which comprises first immersing the fibers in a heated solution of carbonate of soda in a 105 boiler under pressure; drawing off the bath from the boiler and replacing same by a heated bath of slaked lime, bisulfite of soda,

sal-ammoniac, peroxid of sodium and salts of magnesium and subsequently rinsing the fibers in water.

2. A process for converting vegetable fibers into threads of silky appearance consisting in first immersing the fibers in a heated solution of carbonate of soda in a boiler under pressure; drawing off the bath from the boiler and replacing same by a heated bath of slaked lime, bisulfite of soda, sal-ammoniac, peroxid of sodium and salts of magnesium, primarily rinsing the fibers

with warm water in the boiler, removing the fibers from the boiler and immersing them in an acid bath and finally rinsing said 15 fibers in water.

In witness whereof I have signed this specification in the presence of two witnesses.

JEAN MARIE JOSEPH DEBOURG.

Witnesses:

GASTON JEUNIAUX,  
THOS. W. BROWNE.